

# UNITED STATES PATENT OFFICE.

WOOLSEY McA. JOHNSON AND EDWIN W. HALE, OF HARTFORD, CONNECTICUT,  
ASSIGNORS TO THE CONTINUOUS ZINC FURNACE COMPANY, OF HARTFORD,  
CONNECTICUT, A CORPORATION OF CONNECTICUT.

## DUPLEX SMELTING PROCESS.

1,165,371.

Specification of Letters Patent. Patented Dec. 21, 1915.

No Drawing.

Application filed March 16, 1914. Serial No. 825,190.

To all whom it may concern:

Be it known that we, WOOLSEY McA. JOHNSON and EDWIN W. HALE, both citizens of the United States, and both residing at 5 Hartford, in the county of Hartford and State of Connecticut, have invented a new and Improved Duplex Smelting Process, of which the following specification is a full disclosure.

10 In its more comprehensive aspect, this invention formulates a compound or multi-phase process for isolating volatile materials, notably such metals as zinc, from compounds thereof; and it utilizes the more 15 economic portion of either a special or a conventional single-step treatment as a primary-stage partial reduction and separation, and it then utilizes another treatment in the nature of a secondary-stage operation for the extraction of the remnant 20 values.

A primary object of this invention is to create a way, less costly than now known, for deriving zinc from its ores by interrelating standard one-stage externally-fired zinc-retorting methods with electrical or internally-heated smelting methods; and to do so in such a manner that the portions of 25 each method displaying only the higher efficiency factors with relation to the composition 30 of the charge during its course of treatment will be utilized harmoniously, while other less efficient portions will be dispensed with.

35 Another object is to render available a system of ore treatment in which one step will essentially be carried out in an electric furnace and which step will be preceded by certain steps conventional or otherwise, 40 dealing with ores of a high zinc content and which will extract those metallic values involving a higher electric cost of recovery and which will so condition the material as to bring it into the state best adapted for 45 a high-efficiency in the electric furnace step.

This invention was evolved as a result of a due recognition of certain fundamental facts heretofore not adequately grasped or interrelated by those skilled in this art, that 50 is to say, the reduction of zinc ores by dry methods has been commercially successful for a long time in the externally-fired or fuel-heated way, and we have in a semi-commercial way established successfully the

operation of the internally-heated or electrically treated way. Each system has advantages and each has its limitations, but heretofore the gap between the two has not been bridged. The conventional fuel-fired zinc-retort makes the first two-thirds of its 55 spelter with one-third of the total metallurgical effort, and it is in forcing out the last third of its spelter that the remaining two-thirds of the energy is expended. The importance of this has hardly been 60 appreciated or it has been regarded as a necessary evil; and its significance and possibilities in relation to a characteristic of the electrical system was not grasped. This 65 characteristic is that the electrical method attains its highest efficiency on mixtures such as may obtain in the retort during its low-efficiency end-period; *e. g.* an electric zinc furnace operates less economically on a 70 60% zinc charge which is comparatively 75 costly to smelt electrically; although the last-third is cheaper and more effective than corresponding portions of other processes. The adaptability of this duplex process may 80 perhaps be best illustrated by a typical practical application thereof. Assume a Joplin ore of this composition:

(A) 90% ZnS; 2% FeS<sub>2</sub>; 4% SiO<sub>2</sub>; 1% Al<sub>2</sub>O<sub>3</sub>; 2% CaCO<sub>3</sub>.

85 This is a high-grade zinc ore such as is conventionally treated for the ordinary retort process by first roasting to about this composition:

(B) 72% Zn; 1.5% Fe; 4.7% SiO<sub>2</sub>; 1.15% Al<sub>2</sub>O<sub>3</sub>; 3.03% CaSO<sub>4</sub>.

90 Conventionally, also, this ore is then mixed with about 45% of its weight of coal and is introduced into cylindrical retorts 95 and heated at temperatures progressively rising to 1350° C. or over, with a retort life of about 30 days, and the commercially extractable zinc is recovered, leaving a residue that is thrown away, and which analyzes about as follows:

(C) 6% Zn; 5% S; 8% Fe; 25% SiO<sub>2</sub>; 15% Al<sub>2</sub>O<sub>3</sub>; 35% C and 5% CaS.

100 The percentage composition of (C) will depend upon the nature of the reduction coal used and upon the nature of the ash thereof.

Now, this process in such a case would modify this conventional complete treatment by changing it into an incomplete step which would yield a portion only of the metallic values, and which would result in an end-product which, instead of being constituted like C, would be composed somewhat as follows:

10 (D) 20% Zn; 3.5% S; 18% SiO<sub>2</sub>; 30% C; Fe 6%; Al<sub>2</sub>O<sub>3</sub> 10%.

First stage treatment.—To do this, the ore (A) would be roasted to bring it into the composition (B) as before, but if desired 15 higher in sulfur. Preferably however, this roasted material will be mixed with somewhat less coal, say 25%, since the reduction of the metal is not carried to a finality in the retorts. Or, instead of working up to 20 the aforesaid composition (B), this invention permits the employment of a modified starting composition; *i.e.*, one that contains more iron and lime, and therefore which 25 will tend to slag at a lower temperature than the convention composition B. This modification is made possible because this process 30 does not subject the starting composition to temperatures as high as those needed in ordinary retorting. Furthermore, retorts of 35 greater capacity may be employed with advantage, by reason of the moderate temperature of about 1150° C.; thereby keeping loss of zinc by volatilization low due to the moderate temperature, and also avoiding the formation 40 of slag in the retort or causing undue corrosion of the retorts. This also effects a reduction in the "soakage" loss by reason of the decreased discarding of retorts due to their increased life. The moderate 45 temperatures used and the fact that the charge is not forced, makes it feasible to use retorts 11 inches or 12 inches square, instead of 8½ round, and the charge (such as D) now analyzing say 20% zinc with about 30% fixed carbon may easily be "blown out."

In ordinary retorting practice, a difficulty arises at the end of the operation in 50 respect to determining what had best be the finishing temperature and in controlling the final heating so as not to exceed the practically estimated maximum. The reason for this lies in the endothermic character of the 55 reaction



This means that so long as this reaction is taking place, at a substantial rate, the heat absorbed by the reaction is cooling the retort, and when this refrigerating effect abruptly ceases while yet the furnace is under full fire, then the retort contents will attain a destructively high temperature before the operator can sufficiently check the furnace. By our system, however, there need be no

opportunity for this uncontrollable temperature uprise, because the heating is terminated considerably before the end of the endothermic reduction and the operation does not need to hug the danger point.

Second stage treatment.—The second stage treatment will now be applied for the purpose of recovering the metallic values of the residue D, and the preliminary steps of this treatment are for the purpose of preparing the charge for the electric furnace. Preferably, this preparation follows the teachings of the Johnson U. S. Patent No. 868345, granted October 15, 1907, in that the charge is made to contain metallic iron for the purpose of decomposing the zinc sulfid in the electric furnace, and it is so constituted as to enable the furnace to be operated in accordance with the Johnson Canadian Patent No. 146134, granted February 25, 1913.

Thus, the residue D may be mixed with low grade ore analyzing green, say, 15% zinc, 10% lead, 2% copper, 22% iron and 25% sulfur. This green ore will be first roasted to lower its sulfur content to a desired minimum by utilizing the relatively low roasting temperature of 850° to 900° centigrade, the effect of which will be to convert the larger portions of the sulfates of iron and zinc into oxids. It is not necessary to dead-roast this ore as a slight per cent. of sulfur, say from 3 to 6 is necessary. This roasted ore is now, as before stated, mixed with the residue D, and also with such necessary additional fluxes as zinc carbonate (high in lime) or with lime alone, so as to form a complete slagging charge adaptable for continuous operation. It is noteworthy that this mixture contains no hydro-carbons, but only fixed carbon, and accordingly, hydro-carbons are preferably added, either directly to the charge by using a small percentage of coal high in volatile matter and low in fixed carbon, or by incorporating a certain amount of crude oil into charge. This facilitates the operation of the charge in the electric furnace by affording a liberal diffusion of reducing elements throughout the charge. This additional green ore having been first roasted to reduce the sulfur to workable limits, its addition to the retort residue D furnishes the latter with the oxygen necessary to consume its excess of fixed carbon and prevent carbon from accumulating in the electric furnace. This mixture may be represented as follows:

(F) 30% Zn; 12% Fe; 1.5% Cn; 8% CaO; 12% SiO<sub>2</sub>; 4% Al<sub>2</sub>O<sub>3</sub>; 13% C.

The iron oxid in this charge must now be converted into sponge iron to a large extent in the "preheating" or "metallizing" operation. Enough carbon or other reducing agent had been brought into the mixture as above described in percentages sufficiently

high to effect this "metallizing" of the charge. That is to say, about 10% to 15% of carbon, or the exact theoretical amounts, to effect the proper reduction of the oxids 5 present with such an excess as may be necessary to compensate for such accidental or incidental oxidation as may happen in the "metallizing" operation. This may come from the opening of the doors to greater 10 or less extent, or by such leaks as would happen in the ordinary course of events. This second heating or so-called "preheating" or "metallizing" is carried on in a furnace of the muffle type to a final temperature 15 of about 1000° centigrade under reducing conditions. This preliminary pre-heating treatment yields a mixture in accordance with the teachings of the above mentioned patents, and electric smelting of 20 preheating charge is so carried on recovery high percentages of zinc, copper, gold, silver and lead in merchantable form.

The composition D (yielded by the retort after the partial recovery of zinc) may be 25 given slagging characteristics by mixing it with suitable retorted material, instead of with roasted green ore. That is to say, two different non-slagging mixtures, the one acid and the other basic, may be separately retorted 30 either intermittently or continuously and they may thereafter be mixed together in such proportions and if needed with such other side material as will compound a true slagging mixture suitable for smelting in 35 the electric furnace.

Having thus revealed this invention, we claim as new and desire to secure by Letters Patent of the United States:

1. A smelting process of the nature disclosed, consisting in preparing a self-reducing charge; inserting said charge within a suitable retort; externally heating said retort for a sufficient time-period to effect a partial reduction only of the contained 45 charge, and discontinuing the external heating of the charge at a temperature materially short of that essential for a commercially ultimate reduction; and finally completing the reduction to a commercially ultimate extent by means of materially higher 50 temperatures obtained by suitably developing heat within the charge inclosed in a suitable container.

2. A smelting process of the nature disclosed, consisting in preparing a self-reducing mixture; bringing said mixture within a suitable retort; externally heating said retort for a sufficient time and at a sufficient

temperature to effect an incomplete reduction of the mixture and obtain a partial recovery of the metallic value; and finally completing the reduction and effecting a commercially ultimate recovery of the metallic value by suitably developing internal heat within the partially treated mixture at 65 temperatures materially higher than obtained by the external heating.

3. The process revealed for producing a volatile metal consisting in preparing a self-reducing charge containing a compound of 70 said metal; inserting said charge within a suitable retort; externally heating said retort to effect an incomplete reduction of the contained charge, withdrawing the volatilized reduced metal from said retort, and terminating the effective heating of the charge 75 materially short of the point of ultimate commercial reduction; thereafter raising the pre-treated charge inclosed in a suitable container to materially higher temperatures by 80 internally applying heat thereto until the point of ultimate commercial reduction is attained, and meanwhile withdrawing and recovering the volatilized metal.

4. A process for reducing high-grade zinc-ores consisting in obtaining the zinc-bearing material in a state having a low sulfur content, then forming a retort charge thereof by the addition of carbon, then heating said mixture in a retort externally heated to a 90 temperature rising to about 1150° C., as a maximum, thereafter utilizing the residue from said retort together with additional carbon for preparing another mixture, and then obtaining the ultimate metallic values 95 by electrically developing heat within the charge while inclosed in an air-excluding container.

5. A process of the nature revealed for extracting values from zinc ores, which consists in effecting a preliminary partial recovery of metallic zinc by first reducing the zinc-bearing material in externally heated fire-clay retorts under non-slagging conditions, and then applying electric heat under 105 slagging conditions, thereby recovering the residual zinc and other values.

In witness whereof, we hereunto subscribe our names, as attested by the two subscribing witnesses.

WOOLSEY McA. JOHNSON.  
EDWIN W. HALE.

Witnesses:

HENRY H. PEASE,  
CHAS. A. HUNTER.